# EUROPEAN PATENT SPECIFICATION

(11) **EP 2 049 630 B1**
(45) Date of publication and mention of the grant of the patent: **29.04.2015**
(21) Application number: 07787797.5
(22) Date of filing: 23.07.2007
(51) Int. Cl.: C10M 133/06, C10N 30/10, C10N 30/00

(54) **LUBRICANT COMPOSITION**
SCHMIERSTOFFZUSAMMENSETZUNG
COMPOSITION DE LUBRIFIANT

(30) Priority: 31.07.2006 US 834383 P
(43) Date of publication of application: 22.04.2009
(73) Proprietor: BASF SE, 67056 Ludwigshafen (DE)
(72) Inventor: CHASAN, David Eliezer, Teaneck, NJ 07666 (US); WILSON, Patricia Roberta, White Plains, NY 10606 (US); RIBEAUD, Marc, 2800 Delémont (CH)
(74) Representative: Fiesser, Gerold Michael
(86) International application number: PCT/EP2007/057552
(87) International publication number: WO 2008/015116

(56) References cited:
- EP-A- 0 356 677
- WO-A-02/04578
- JP-A- 60 028 496
- US-A- 5 268 113
- US-A- 5 273 669
- DOBRESCU V ET AL: "THE ANTIOXIDIZING EFFECT OF STERICALLY HINDERED AMINES IN THERMAL OXIDATION OF LOW DENSITY POLYETHYLENE" EUROPEAN POLYMER JOURNAL, PERGAMON PRESS LTD. OXFORD, GB, vol. 24, no. 3, 1988, pages 289-294, XP002033506 ISSN: 0014-3057

## Description

The present invention relates to lubricant compositions stabilized against oxidative degradation via the incorporation of certain sterically hindered amine stabilizers. The lubricant compositions exhibit excellent results regarding seal swell.

U.S. Pat. Nos. 5,073,278 and 5,273,669 teach the stabilization of lubricant compositions with a certain aromatic amine and at least one sterically hindered amine.

U.S. Pat. No. 5,268,113 discloses lubricants stabilized by the addition of a sterically hindered amine and a phenol. EP 0356677 discloses lubricants comprising a mineral or synthetic base oil, an aromatic amine and at least one sterically hindered amine. International Application WO 02/04578 discloses lubricant compositions including blends of Group II and/or Group III base oils and alkylated aromatic compositions which exhibit excellent additive solvency, thermo-oxidative stability, hydrolytic stability, and seal swell characteristics.

It is known to add stabilizers to lubricants based on mineral or synthetic oils in order to improve their performance characteristics. Antioxidants are of particular importance. Oxidative degradation of lubricants plays a significant role especially in motor oils because of the high temperatures prevailing in the combustion chambers of the engines and the presence, in addition to oxygen, of oxides of nitrogen which act as oxidation catalysts.

Hindered amine compounds are effective stabilizers for lubricants. However, they are generally not employed due to detrimental effects such as seal swell.

The present invention relates to the stabilization of lubricant compositions with a specific class of hindered amine compounds. The present lubricant compositions are non-aggressive towards seals.

The present invention relates to a stabilized lubricant composition which comprises

A mineral or a synthetic base oil or a mixture of a mineral and a synthetic base oil; and

At least one sterically hindered amine compound of the formula where R is a straight or branched alkyl group of 7, 8, 9, 10, 11, 12, 13, 14, 15 or 16.

The sterically hindered amines are known and are prepared according to methods known in the art. For example, the present hindered amines are 2,2,6,6-tetramethylpiperidin-4-ol esters of aliphatic carboxylic acids, for example the esters of lauric acid or stearic acid.

According to a preferred embodiment, the invention relates to compositions wherein the hindered amines of the formula is present.

Lubricants according to the present invention are functional fluids, that is lubricants, hydraulic fluids or metal working fluids.

Lubricants are in particular mineral oil based (API classifications Groups I, II, III, Group IV including gas to liquid (GTL) oils) or synthetic base oils, such as is normally used for the production of lubricants. Synthetic oils may be, for example, esters of polycarboxylic acids or of polyols; they may also be aliphatic polyesters or poly-α-olefins, silicones, phosphoric acid esters or polalkylene glycols. The lubricant may also be a grease based on an oil and a thickener. Such lubricants are described, for example in D. Klamann "Schmierstoffe und artverwandte Producte", Verlag Chemie, Weinheim, 1982.

Examples are lubricants and hydraulic fluids based on mineral oil or synthetic lubricants or hydraulic fluids, in particular those which are derivatives of carboxylic esters and which are used at temperatures of 200°C and above.

Examples of synthetic lubricants embrace lubricants based on a diester of a dibasic acid with a monovalent alcohol, for example dioctyl sebacate or dinonyl adipate, a triester of trimethylolpropane with a monobasic acid or a mixture of such acids, for example trimethylolpropane tripelargonate, trimethylolpropane tricaprylate or mixtures of these, a tetraester of pentaerythritol with a monobasic acid or with a mixture of such acids, for example pentaerythritol tetracaprylate, or a complex ester of monobasic and dibasic acids with polyhydric alcohols, for example a complex ester of trimethylolpropane with caprylic and sebacic acid or a mixture of these.

Particularly suitable are, besides mineral oils, for example poly-α-olefins, lubricants based on esters, or phosphates, glycols, polyglycols and polalkyene glycols and mixtures of these with water.

The sterically hindered amines of this invention are in particular non-aggressive toward elastomeric seals.

The seals are in particular a fluoropolymer elastomer used in O-rings and other goods. The "fluoroelastomers" are categorized under ASTM D1418 and ISO 1629 designation of FKM for example. The fluoroelastomers comprise copolymers of hexafluoropropylene (HFP) and vinylidene fluoride (VDF of VF2), terpolymers of tetrafluoroethylene (TFE), vinylidene fluoride and hexafluoropropylene, perfluoromethylvinylether (PMVE), copolymers of TFE and propylene and copolymers of TFE, PMVE and ethylene. The fluorine content varies for example between about 66 to about 70% by weight.

FKM is fluoro rubber of the polymethylene type having substituent fluoro and perflouroalkyl or perfluoroalkoxy groups on the polymer chain.

Accordingly, a preferred subject of the invention is a method which comprises contacting a fluoroelastomer with a stabilized lubricant composition, which comprises
At least one mineral or a synthetic base oil or a mixture of a mineral and a synthetic base oil and
At least one or more sterically hindered amine compounds of the formula (I), where R is a straight or branched alkyl group of 7, 8, 9, 10, 11, 12, 13, 14, 15 or 16.

The sterically hindered amines according to this invention are admixed with the lubricants in an amount of about 0.01 to about 5% by weight, for example from about 0.05 to about 3% by weight, for instance from about 0.1 to about 2% by weight, based on the weight of the lubricant.

The lubricants can additionally comprise other additives which are added to improve the basic properties of lubricants even further; these include antioxidants, metal passivators, rust inhibitors, viscosity index improvers, pour point depressors, dispersants, detergents, high pressure additives, antifriction additives and antiwear additives.

These additional additives are for example:
1. Antioxidants
1.1. Alkylated monophenols, for example 2,6-di-tert-butyl-4-methylphenol, 2-tert-butyl -4,6-dimethylphenol, 2,6-di-tert-butyl-4-ethylphenol, 2,6-di-tert-butyl-4-n-butylphenol, 2,6-di-tert-butyl-4-isobutylphenol, 2,6-dicyclopentyl-4-methylphenol, 2-(α-methylcyclohexyl)-4,6-dimethylphenol, 2,6-dioctadecyl-4-methylphenol, 2,4,6-tricyclohexylphenol, 2,6-di-tert-butyl-4-meth-oxymethylphenol, 2,6-di-nonyl-4-methylphenol, 2,4-dimethyl -6(1'-methylundec-1'-yl)phenol, 2,4-dimethyl-6-(1'-methylheptadec-1'-yl)phenol, 2,4-dimethyl-6-(1'-methyltridec-1'-yl)phenol and mixtures thereof.
1.2. Alkylthiomethylphenols, for example 2,4-dioctylthiomethyl-6-tert-butylphenol, 2,4-dioc-tylthiomethyl-6-methylphenol, 2,4-dioctylthiomethyl-6-ethylphenol, 2,6-didodecylthiomethyl-4-nonylphenol.
1.3. Hydroquinones and alkylated hydroquinones, for example 2,6-di-tert-butyl-4-methoxyphenol, 2,5-di-tert-butylhydroquinone, 2,5-di-tert-amylhydroquinone, 2,6-diphenyl-4-octade-cyloxyphenol, 2,6-di-tert-butylhydroquinone, 2,5-di-tert-butyl-4-hydroxyanisole, 3,5-di-tert-butyl-4-hydroxyanisole, 3,5-di-tert-butyl-4-hydroxyphenyl stearate, bis-(3,5-di-tert-butyl-4-hy-droxyphenyl) adipate.
1.4. Hydroxylated thiodiphenyl ethers, for example 2,2'-thiobis(6-tert-butyl-4-methylphenol), 2,2'-thiobis(4-octylphenol), 4,4'-thiobis(6-tert-butyl-3-methylphenol), 4,4'-thiobis(6-tert-butyl-2-methylphenol), 4,4'-thiobis-(3,6-di-sec-amylphenol), 4,4'-bis-(2,6-dimethyl-4-hydroxyphenyl) disulfide.
1.5. Alkylidenebisphenols, for example 2,2'-methylenebis(6-tert-butyl-4-methylphenol), 2,2'-methylenebis(6-tert-butyl-4-ethylphenol), 2,2'-methylenebis[4-methyl-6-(α-methylcyclohexyl)phenol], 2,2'-methylenebis(4-methyl-6-cyclohexylphenol), 2,2'-methylenebis(6-nonyl-4-methylphenol), 2,2'-methylenebis(4,6-di-tert-butylphenol), 2,2'-ethylidenebis (4,6-di-tert-butyl-phenol), 2,2'-ethylidenebis(6-tert-butyl-4-isobutylphenol), 2,2'-methylenebis [6-(α-methylben-zyl)-4-nonyl phenol], 2,2'-methylenebis[6-(α,α-dimethylbenzyl) -4-nonylphenol], 4,4'-methyle-nebis(2,6-di-tert-butylphenol), 4,4'-methylenebis(6-tert-butyl-2-methylphenol),1,1-bis(5-tert-butyl-4-hydr oxy-2-methylphenyl)butane, 2,6-bis(3-tert-butyl-5-methyl-2-hydroxybenzyl)-4-methylphenol, 1,1,3-tris(5-tert-butyl-4-hydroxy-2-methylphenyl)butane, 1,1-bis(5-tert-butyl-4-hydroxy-2-methyl-phenyl)-3-n-dodecylmercaptobutane, ethylene glycol bis[3,3-bis(3'-tert-bu-tyl-4'-hydroxyphenyl)butyrate], bis(3-tert-butyl-4-hydroxy-5-methyl-phenyl)dicyclopentadiene, bis[2-(3'-tert-butyl -2'-hydroxy-5'-methylbenzyl) -6-tert-butyl-4-methylphenyl]terephthalate, 1,1-bis-(3,5-dimethyl-2-hydroxyphenyl)butane, 2,2-bis-(3,5-di-tert-butyl-4-hydroxyphenyl)propane, 2,2-bis-(5-tert-butyl-4-hydroxy2-methylphenyl)-4-n-dodecylmercaptobutane, 1,1,5,5-tetra-(5-tert -butyl-4-hydroxy2-methylphenyl)pentane.
1.6. O-, N- and S-benzyl compounds, for example 3,5,3',5'-tetra-tert-butyl-4,4'-dihydroxy-dibenzyl ether, octadecyl-4-hydroxy-3,5-dimethylbenzylmercaptoacetate, tris-(3,5-di-tert -bu-tyl-4-hydroxybenzyl)amine, bis(4-tert-butyl-3-hydroxy-2,6-dimethylbenzyl)dithioterephthalate, bis(3,5-di-tert-butyl-4-hydroxybenzyl)sulfide, isooctyl-3,5di-tert-butyl-4-hydroxybenzylmer-captoacetate.
1.7. Hydroxybenzylated malonates, for example dioctadecyl-2,2-bis-(3,5-di-tert-butyl-2-hy-droxybenzyl)-malonate, di-octadecyl-2-(3-tert-butyl-4-hydroxy-5-methylbenzyl)-malonate, di-dodecylmercaptoethyl-2,2-bis-(3,5-di-tert-butyl-4-hydroxybenzyl)malonat e, bis [4-(1,1,3,3-tetramethylbutyl)phenyl]-2,2-bis(3,5-di-tert-butyl-4-hydroxybe nzyl)malonate.
1.8. Aromatic hydroxybenzyl compounds, for example 1,3,5-tris-(3,5-di-tert-butyl-4-hydroxybenzyl)-2,4,6-trimethylbenzene, 1,4-bis(3,5-di-tert-butyl-4-hydroxybenzyl)-2,3,5,6-tetramethylbenzene, 2,4,6-tris(3,5-di-tert-butyl-4-hydroxybenzyl)phenol.
1.9. Triazine Compounds, for example 2,4-bis(octylmercapto)-6-(3,5-di-tert-butyl-4-hy-droxyanilino)-1,3,5-triazine, 2-octylmercapto-4,6-bis(3,5-di-tert-butyl-4-hydroxyanilino) -1,3,5-triazine, 2-octylmercapto-4,6-bis(3,5-di-tert-butyl-4-hydroxyphenoxy)-1,3,5-triazine, 2,4,6-tris(3,5-di-tert-butyl-4-hydroxyphenoxy)-1,2,3-triazine, 1,3,5-tris(3,5-di-tert-butyl-4-hydroxy-benzyl)isocyanurate, 1,3,5-tris(4-tert-butyl-3-hydroxy-2,6-dimethylbenzyl 2,4,6-tris(3,5-di-tert-butyl-4-hydroxyphenylethyl)-1,3,5-triazine, 1,3,5-tris(3,5-di-tert-butyl-4-hydroxyphenylpropio-nyl)-hexahydro-1,3,5-triazine, 1,3,5-tris(3,5-dicyclohexyl-4-hydroxybenzyl)isocyanurate.
1.10. Benzylphosphonates, for example dimethyl-2,5-di-tert-butyl-4-hydroxybenzylphospho-nate, diethyl-3,5-di-tert-butyl-4-hydroxybenzylphosphonate, dioctadecyl3,5-di-tert-butyl-4-hydroxybenzylphosphonate, dioctadecyl-5-tert-butyl-4-hydroxy3-methylbenzylphosphonate, the calcium salt of the monoethyl ester of 3,5-di-tert-butyl-4-hydroxybenzylphosphonic acid.
1.11. Acylaminophenols, for example 4-hydroxylauranilide, 4-hydroxystearanilide, octyl N-(3,5-di-tert-butyl-4-hydroxyphenyl)carbamate.
1.12. Esters of [3-(3,5-di-tert-butyl-4-hydroxyphenyl)propionic acid with mono- or polyhydric alcohols, e.g. with methanol, ethanol, octadecanol, 1,6-hexanediol, 1,9-nonanediol, ethylene glycol, 1,2-propanediol, neopentyl glycol, thiodiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2,6,7-trioxabicyclo[2.2.2]octane.
1.13. Esters of β-(5-tert-butyl-4-hydroxy-3-methylphenyl)propionic acid with mono- or polyhydric alcohols, e.g. with methanol, ethanol, octadecanol, 1,6-hexanediol, 1,9-nonanediol, ethylene glycol, 1,2-propanediol, neopentyl glycol, thiodiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2,6,7-trioxabicyclo[2.2.2]octane.
1.14 Esters of 13-(3,5-dicyclohexyl-4-hydroxyphenyl)propionic acid with mono- or polyhydric alcohols, e.g. with methanol, ethanol, octadecanol, 1,6-hexanediol, 1,9-nonanediol, ethylene glycol, 1,2-propanediol, neopentyl glycol, thiodiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2,6,7-trioxabicyclo[2.2.2]octane.
1.15 Esters of 3,5-di-tert-butyl-4-hydroxyphenyl acetic acid with mono- or polyhydric alcohols, e.g. with methanol, ethanol, octadecanol, 1,6-hexanediol, 1,9-nonanediol, ethylene glycol, 1,2-propanediol, neopentyl glycol, thiodiethylene glycol, diethylene glycol, triethylene glycol, pentaerythritol, tris(hydroxyethyl) isocyanurate, N,N'-bis(hydroxyethyl)oxamide, 3-thiaundecanol, 3-thiapentadecanol, trimethylhexanediol, trimethylolpropane, 4-hydroxymethyl-1-phospha-2,6,7-trioxabicyclo[2.2.2]octane.
1.16. Amides of β-(3,5-di-tert-butyl-4-hydroxyphenyl)propionic acid e.g. N,N'-bis(3,5-di-tert-butyl-4-hydroxyphenylpropionyl)hexamethylenediamine, N,N'-bis(3,5-di-tert-butyl -4-hydroxy-phenylpropionyl)trimethylenediamine, N,N'-bis(3,5-di-tert-butyl-4-hydroxyphenylpropio-nyl)hydrazine.

### Aminic antioxidants:

N,N'-diisopropyl-p-phenylenediamine, N,N'-di-sec-butyl-p-phenylenediamine, N,N'-bis (1,4-dimethylpentyl)-p-phenylenediamine, N,N'-bis(1-ethyl-3-methylpentyl)-p-phenylenediamine, N,N'-bis(1-methylheptyl)-p-phenylenediamine, N,N'-dicyclohexyl-p-phenylenediamine, N,N'-diphenyl-p-phenylenediamine, N,N'-bis(2-naphthyl)-p-phenylenediamine, N-isopropyl-N'-phenyl-p-phenylenediamine, N-(1,3-dimethyl-butyl)-N'-phenyl-p-phenylenediamine, N-(1-methylheptyl)-N'-phenyl-p-phenylenediamine, N-cyclohexyl-N'-phenyl-p-phenylenediamine, 4-(p-toluenesulfamoyl)diphenylamine, N,N'-dimethyl-N,N'-di-sec-butyl-p-phenylenediamine, diphenylamine, N-allyldiphenylamine, 4-isopropoxydiphenylamine, N-phenyl-1-naphthylamine, N-phenyl-2-naphthylamine, octylated diphenylamine, for example p,p'-di-tert-octyldi-phenylamine, 4-n-butylaminophenol, 4-butyrylaminophenol, 4-nonanoylaminophenol, 4-do-decanoylaminophenol, 4-octadecanoylaminophenol, bis(4-methoxyphenyl)amine, 2,6-di-tert-butyl-4-dimethylaminomethylphenol, 2,4'-diaminodiphenylmethane, 4,4'-diaminodiphenyl-methane, N,N,N',N'-tetramethyl -4,4'-diaminodiphenylmethane, 1,2-bis[(2-methyl-phenyl)amino]ethane, 1,2-bis(phenylamino)propane, (o-tolyl)biguanide, bis[4-(1',3'-dimethyl-butyl)phenyl]amine, tert-octylated N-phenyl-1-naphthylamine, a mixture of mono- and dialkylated tert-butyl/tert-octyldiphenylamines, a mixture of mono- and dialkylated isopropyl/isohexyldiphenylamines, mixtures of mono- and dialkylated tert-butyldiphenylamines, 2,3-dihydro-3,3-dimethyl-4H-1,4-benzothiazine, phenothiazine, N-allylphenothiazine, N,N,N',N'-tetraphenyl -1,4-diaminobut-2-ene, N,N-bis(2,2,6,6-tetramethylpiperid-4-yl-hexamethyl-enediamine, bis(2,2,6,6 -tetramethylpiperid-4-yl)sebacate, 2,2,6,6-tetramethylpiperidin-4-one and 2,2,6,6-tetramethylpiperidin-4-ol.

### Examples of other antioxidants:

Aliphatic or aromatic phosphites, esters of thiodipropionic acid or of thiodiacetic acid, or salts of dithiocarbamic or dithiophosphoric acid, 2,2,12,12-tetramethyl-5,9-dihydroxy -3,7,11 - trithiatridecane and 2,2,15,15- tetramethyl-5,12-dihydroxy-3,7,10,14-tetrathiahexadecane. Examples of metal deactivators, for example for copper, are:
a) Benzotriazoles and derivatives thereof, for example 4- or 5-alkylbenzotriazoles (e.g. tolutriazole) and derivatives thereof, 4,5,6,7-tetrahydrobenzotriazole and 5,5'-methylenebisben-zotriazole; Mannich bases of benzotriazole or tolutriazole, e.g. 1-[bis(2-ethylhexyl)aminomethyl)tolutriazole and 1-[bis(2-ethylhexyl)aminomethyl)benzotriazole; and alkoxyalkylbenzotriazoles such as 1-(nonyloxymethyl)benzotriazole, 1-(1 -bu-toxyethyl)benzotriazole and 1-(1-cyclohexyloxybutyl)tolutriazole.
b) 1,2,4-Triazoles and derivatives thereof, for example 3-alkyl(or aryl)-1,2,4-triazoles, and Mannich bases of 1,2,4-triazoles, such as 1-[bis(2-ethylhexyl)aminomethyl -1,2,4-triazole; alkoxyalkyl-1,2,4-triazoles such as 1-(1-butoxyethyl)-1,2,4-triazole; and acylated 3-amino-1,2,4-triazoles.
c) Imidazole derivatives, for example 4,4'-methylenebis(2-undecyl-5-methylimidazole) and bis[(N-methyl)imidazol-2-yl]carbinol octyl ether.
d) Sulfur-containing heterocyclic compounds, for example 2-mercaptobenzothiazole, 2,5-dimercapto-1,3,4-thiadiazole and derivatives thereof; and 3,5-bis[di(2-ethylhexyl)aminomethyl]-1,3,4-thiadiazolin-2-one.
e) Amino compounds, for example salicylidenepropylenediamine, salicylaminoguanidine and salts thereof.

### Examples of rust inhibitors and friction modifiers are:

a) Organic acids, their esters, metal salts, amine salts and anhydrides, for example alkyl- and alkenylsuccinic acids and their partial esters with alcohols, diols or hydroxycarboxylic acids, partial amides of alkyl- and alkenylsuccinic acids, 4-nonylphenoxyacetic acid, alkoxy- and alkoxyethoxycarboxylic acids such as dodecyloxyacetic acid, dodecyloxy(ethoxy)acetic acid and the amine salts thereof, and also N-oleoylsarcosine, sorbitan monooleate, lead naphthenate, alkenylsuccinic anhydrides, for example dodecenylsuccinic anhydride, 2-car-boxymethyl-1-dodecyl-3-methylglycerol and the amine salts thereof.
b) Nitrogen-containing compounds, for example:
   I. Primary, secondary or tertiary aliphatic or cycloaliphatic amines and amine salts of organic and inorganic acids, for example oil-soluble alkylammonium carboxylates, and also 1-[N,N-bis(2-hydroxyethyl)amino]-3-(4-nonylphenoxy)propan-2-ol.
   II. Heterocyclic compounds, for example: substituted imidazolines and oxazolines, and 2-heptadecenyl-1-(2-hydroxyethyl)imidazoline.
c) Phosphorus-containing compounds, for example: Amine salts of phosphoric acid partial esters or phosphonic acid partial esters, and zinc dialkyldithiophosphates.
d] Molybdenum- containing compounds, such as Molydbenum dithiocarbamate and other sulphur and phosphorus containing derivatives
e) Sulfur-containing compounds, for example: barium dinonylnaphthalenesulfonates, calcium petroleum sulfonates, alkylthio-substituted aliphatic carboxylic acids, esters of aliphatic 2-sulfocarboxylic acids and salts thereof.
f) Glycerol derivatives, for example: glycerol monooleate, 1-(alkylphenoxyy3-(2-hydroxyethyl)glycerols, 1-(alkylphenoxy)-3-(2,3-dihydroxypropyl)glycerols and 2-carboxyalkyl-1,3-dialkylglycerols.

Examples of viscosity index improvers are:
Polyacrylates, polymethacrylates, vinylpyrrolidone/methacrylate copolymers, polyvinylpyrroli-dones, polybutenes, olefin copolymers, styrene/acrylate copolymers and polyethers.

Examples of pour-point depressants are:
Polymethacrylate and alkylated naphthalene derivatives.

Examples of dispersants/surfactants are:
Polybutenylsuccinic amides or -imides, polybutenylphosphonic acid derivatives and basic magnesium, calcium and barium sulfonates and phenolates.

Examples of antiwear additives are:
Sulfur- and/or phosphorus- and/or halogen-containing compounds, e.g. sulfurised olefins and vegetable oils, zinc dialkyldithiophosphates, alkylated triphenyl phosphates, tritolyl phosphate, tricresyl phosphate, chlorinated paraffins, alkyl and aryl di- and trisulfides, amine salts of mono- and dialkyl phosphates, amine salts of methylphosphonic acid, diethanolami-nomethyltolyltriazole, bis(2-ethylhexyl)aminomethyltolyltriazole, derivatives of 2,5-dimer-capto-1,3,4-thiadiazole, ethyl 3-[(diisopropoxyphosphinothioyl)thio]propionate, triphenyl thiophosphate (triphenylphosphorothioate), tris(alkylphenyl) phosphorothioate and mixtures thereof (for example tris(isononylphenyl) phosphorothioate), diphenyl monononylphenyl phosphorothioate, isobutylphenyl diphenyl phosphorothioate, the dodecylamine salt of 3-hy-droxy-1,3-thiaphosphetane 3-oxide, trithiophosphoric acid 5,5,5-tris[isooctyl 2-acetate], derivatives of 2-mercaptobenzothiazole such as 1-[N,N-bis (2-ethylhexyl)aminomethyl]-2-mer-capto-1H-1,3-benzothiazole, and ethoxycarbonyl-5-octyldithiocarbamate.

The examples which follow illustrate the invention in greater detail. Parts and percentages are by weight, unless otherwise indicated.

### Example

The superiority of the claimed sterically hindered amines over other similar sterically hindered amine additives is illustrated by the following example. A 5W-30 engine oil containing 0.08 %P is supplemented with sufficient sterically hindered amine additive to raise the total base number, as measured by ASTM D 4739 by two units. Amine additive A is added at a treat level of 1.0 weight percent and amine additive B is added at a treat level of 1.2%. The oils are stirred at 60°C for one hour to insure homogeneity. The formulations are tested according to elastomer compatibility procedure CEC- L-39-T-96. The results of the CEC- L-39-T-96 testing of these formulations with an FKM fluorinated rubber are found below. Both amines affected the rubber elastomer.

| **Material** | **1** wt% | **2** wt% | **3** wt% | |
|---|---|---|---|---|
| Base formulation | 100 | 99.0 | 98.8 | |
| Amine A (comparative amine) | 0 | 1.0 | 0 | |
| Amine B (according to the invention) | 0 | 0 | 1.2 | |

| **Results** | | | | |
|---|---|---|---|---|
| FKM rubber | | | | ACEA Spec |
| Hardness [DIDC, points] | -1 | 3 | 0 | -1/+5 |
| Tensile strength [%] | -17 | -51 | -33 | -40/+10 |
| Elongation at rupture [%] | -29 | -75 | -55 | -5-/+10 |
| Volume variation [%] | 0.7 | 1.1 | 1.1 | -1/+5 |

The magnitude of the effect of amine A on tensile strength and elongation at rupture made it totally unsuitable for use relative to specifications such as that of ACEA. Amine B has much less of an effect on the fluorinated rubber- indicating it is suitable for use in engine oils.

Amine A is

Amine B is

## Claims

1. A stabilized lubricant composition which comprises
A mineral or a synthetic base oil or a mixture of a mineral and a synthetic base oil and At least one sterically hindered amine compound of the formula where R is a straight or branched alkyl group of 7, 8, 9, 10, 11, 12, 13, 14, 15 or 16 carbon atoms.

2. A composition according to claim 1 where R is a straight or branched alkyl group of 11 carbon atoms.

3. A composition according to claim 1 where the hindered amine is of the formula

4. A composition according to claim 1 where the hindered amine is present from about 0.01 to about 5% by weight, based on the weight of the lubricant.

5. A composition according to claim 1 where the hindered amine is present from about 0.05 to about 3% by weight, based on the weight of the lubricant.

6. A composition according to claim 1 where the hindered amine is present from about 0.1 to about 2% by weight, based on the weight of the lubricant.

7. A method which comprises
contacting a fluoroelastomer with a stabilized lubricant composition, which comprises At least one mineral or a synthetic base oil or a mixture of a mineral and a synthetic base oil and
At least one or more sterically hindered amine compounds of the formula where R is a straight or branched alkyl group of 7, 8, 9, 10, 11, 12, 13, 14, 15 or 16 carbon atoms.

8. A composition according to claim 1 where R is a straight or branched alkyl group of 8, 9, 10, 11, 12, 13 or 14 carbon atoms.

9. A composition according to claim 1 where R is a straight or branched alkyl group of 10, 11, 12, 13 or 14 carbon atoms.

10. A composition according to claim 1 where R is a straight or branched alkyl group of 10, 11 or 12 carbon atoms.

11. A composition according to claim 1 where R is a straight or branched alkyl group of 11 carbon atoms.

12. A method according to claim 7 where R is a straight or branched alkyl group of 8, 9, 10, 11, 12, 13 or 14 carbon atoms.

13. A method according to claim 7 where R is a straight or branched alkyl group of 10, 11, 12 or 13 carbon atoms.

14. A method according to claim 7 where R is a straight or branched alkyl group of 10, 11 or 12 carbon atoms.

15. A method according to claim 7 where R is a straight or branched alkyl group of 11 carbon atoms.

## Patentansprüche

1. Stabilisierte Schmiermittelzusammensetzung, die ein mineralisches oder synthetisches Grundöl oder eine Mischung aus einem mineralischen und einem synthetischen Grundöl und
mindestens eine sterisch gehinderte Aminverbindung der Formel wobei R für eine gerade oder verzweigte Alkylgruppe mit 7, 8, 9, 10, 11, 12, 13, 14, 15 oder 16 Kohlenstoffatomen steht,
umfasst.

2. Zusammensetzung nach Anspruch 1, wobei R für eine gerade oder verzweigte Alkylgruppe mit 11 Kohlenstoffatomen steht.

3. Zusammensetzung nach Anspruch 1, wobei das gehinderte Amin die Formel aufweist.

4. Zusammensetzung nach Anspruch 1, wobei das gehinderte Amin in einer Menge von etwa 0,01 bis etwa 5 Gew.-%, bezogen auf das Gewicht des Schmiermittels, vorliegt.

5. Zusammensetzung nach Anspruch 1, wobei das gehinderte Amin in einer Menge von etwa 0,05 bis etwa 3 Gew.-%, bezogen auf das Gewicht des Schmiermittels, vorliegt.

6. Zusammensetzung nach Anspruch 1, wobei das gehinderte Amin in einer Menge von etwa 0,1 bis etwa 2 Gew.-%, bezogen auf das Gewicht des Schmiermittels, vorliegt.

7. Verfahren, bei dem man
ein Fluorelastomer mit einer stabilisierten Schmiermittelzusammensetzung, die
mindestens ein mineralisches oder synthetisches Grundöl oder eine Mischung aus einem mineralischen und einem synthetischen Grundöl und
mindestens eine sterisch gehinderte Aminverbindung der Formel wobei R für eine gerade oder verzweigte Alkylgruppe mit 7, 8, 9, 10, 11, 12, 13, 14, 15 oder 16 Kohlenstoffatomen steht,
umfasst, in Berührung bringt.

8. Zusammensetzung nach Anspruch 1, wobei R für eine gerade oder verzweigte Alkylgruppe mit 8, 9, 10, 11, 12, 13 oder 14 Kohlenstoffatomen steht.

9. Zusammensetzung nach Anspruch 1, wobei R für eine gerade oder verzweigte Alkylgruppe mit 10, 11, 12, 13 oder 14 Kohlenstoffatomen steht.

10. Zusammensetzung nach Anspruch 1, wobei R für eine gerade oder verzweigte Alkylgruppe mit 10, 11 oder 12 Kohlenstoffatomen steht.

11. Zusammensetzung nach Anspruch 1, wobei R für eine gerade oder verzweigte Alkylgruppe mit 11 Kohlenstoffatomen steht.

12. Verfahren nach Anspruch 7, wobei R für eine gerade oder verzweigte Alkylgruppe mit 8, 9, 10, 11, 12, 13 oder 14 Kohlenstoffatomen steht.

13. Verfahren nach Anspruch 7 wobei R für eine gerade oder verzweigte Alkylgruppe mit 10, 11, 12 oder 13 Kohlenstoffatomen steht.

14. Verfahren nach Anspruch 7, wobei R für eine gerade oder verzweigte Alkylgruppe mit 10, 11 oder 12 Kohlenstoffatomen steht.

15. Verfahren nach Anspruch 7, wobei R für eine gerade oder verzweigte Alkylgruppe mit 11 Kohlenstoffatomen steht.

## Revendications

1. Composition de lubrifiant stabilisée qui comprend
une huile de base minérale ou synthétique ou un mélange d'une huile de base minérale et synthétique et
au moins un composé d'amine stériquement encombrée de la formule où R est un groupe alkyle linéaire ou ramifié de 7, 8, 9, 10, 11, 12, 13, 14, 15 ou 16 atomes de carbone.

2. Composition selon la revendication 1 dans laquelle R est un groupe alkyle linéaire ou ramifié de 11 atomes de carbone.

3. Composition selon la revendication 1 dans laquelle l'amine encombrée répond à la formule

4. Composition selon la revendication 1 dans laquelle l'amine encombrée est présente à environ 0,01 à environ 5 % en poids, rapporté au poids du lubrifiant.

5. Composition selon la revendication 1 dans laquelle l'amine encombrée est présente à environ 0,05 à environ 3 % en poids, rapporté au poids du lubrifiant.

6. Composition selon la revendication 1 dans laquelle l'amine encombrée est présente à environ 0,1 à environ 2 % en poids, rapporté au poids du lubrifiant.

7. Procédé qui comprend
la mise en contact d'un élastomère fluoré avec une composition de lubrifiant stabilisée, qui comprend
au moins une huile de base minérale ou synthétique ou un mélange d'une huile de base minérale et synthétique et
au moins un ou plusieurs composés d'amine stériquement encombrée de la formule où R est un groupe alkyle linéaire ou ramifié de 7, 8, 9, 10, 11, 12, 13, 14, 15 ou 16 atomes de carbone.

8. Composition selon la revendication 1 dans laquelle R est un groupe alkyle linéaire ou ramifié de 8, 9, 10, 11, 12, 13 ou 14 atomes de carbone.

9. Composition selon la revendication 1 dans laquelle R est un groupe alkyle linéaire ou ramifié de 10, 11, 12, 13 ou 14 atomes de carbone.

10. Composition selon la revendication 1 dans laquelle R est un groupe alkyle linéaire ou ramifié de 10, 11 ou 12 atomes de carbone.

11. Composition selon la revendication 1 dans laquelle R est un groupe alkyle linéaire ou ramifié de 11 atomes de carbone.

12. Procédé selon la revendication 7 dans lequel R est un groupe alkyle linéaire ou ramifié de 8, 9, 10, 11, 12, 13 ou 14 atomes de carbone.

13. Procédé selon la revendication 7 dans lequel R est un groupe alkyle linéaire ou ramifié de 10, 11, 12 ou 13 atomes de carbone.

14. Procédé selon la revendication 7 dans lequel R est un groupe alkyle linéaire ou ramifié de 10, 11 ou 12 atomes de carbone.

15. Procédé selon la revendication 7 dans lequel R est un groupe alkyle linéaire ou ramifié de 11 atomes de carbone.
